

Apr. 10, 1923.

1,451,335

G. R. HANKS

GRINDING BODY AND METHOD OF PRODUCING SAME

Filed Dec. 30, 1921



331

George R. Hanks  
J. S. Richmond

Attorney

Inventor

## UNITED STATES PATENT OFFICE.

GEORGE R. HANKS, OF HIGH BRIDGE, NEW JERSEY, ASSIGNOR TO TAYLOR-WHARTON IRON AND STEEL COMPANY, OF HIGH BRIDGE, NEW JERSEY, A CORPORATION OF NEW JERSEY.

## GRINDING BODY AND METHOD OF PRODUCING SAME.

Application filed December 30, 1921. Serial No. 525,950.

To all whom it may concern:

Be it known that I, GEORGE R. HANKS, a citizen of the United States, residing at High Bridge, in the county of Hunterdon 5 and State of New Jersey, have invented certain new and useful Improvements in Grinding Bodies and Methods of Producing Same, of which the following is a specification.

Objects of my invention are to provide for 10 the rapid production of bodies intended for grinding purposes; to provide for the production of grinding balls free from piping and flashing; and to provide a continuous method of production which will, at one 15 heat, form the slug or blank, densify the same to the ultimate or ball shape, and finally impart the necessary wear and shock resistive properties by appropriate heat treatment.

20 The invention will first be described in connection with the accompanying drawings forming a part hereof, and will then be defined in the claims.

In said drawings,—

25 Figure 1 is a general view of apparatus suitable for use in practicing the invention. Fig. 2 is an elevational view of a ball slug. Fig. 3 is a similar view of a modification; and

30 Fig. 4 is a perspective view of a finished ball.

According to my invention, molten metal is poured into a mold designed to produce a 35 slug a substantial portion of which is of the ultimate shape of the finished grinding body, and the remaining portion of which contains a predetermined amount of metal to complete the article. In short, I provide for a 40 minimum displacement of metal and thus obviate objectionable flashing, regardless of whether the displacement is effected by a hammer or in a press.

The slug may be half spherical as at *a* in Fig. 2, with an offset displaceable portion *b*, the part *a* fitting one of the dies of a suitable forging mechanism, while the offset portion may be of frusto-conical or tapered form. I sometimes, however, make a slug 45 such as is shown at *c* in Fig. 3, in which while maintaining a part contoured to fit the die *d*, the latter is required to cooperate in the forging operation by the extension of the slug in straight lines spaced from the side walls of the die. In either event there is a

predetermined amount of metal to be displaced and there is no flashing.

In the layout, Fig. 1, a ladle 5 carried by an overhead crane 6 serves molten metal to a travelling chain of molds 7, each of which forms a slug 8 of the character indicated. 60 The molds are parted in the usual manner, and as the chain advances the slugs fall into a runway 9 and are delivered in any appropriate manner to a die or displacing mechanism 10. The latter may form an element of a press or of a hammer. In either case the slug 8 adapts itself to the lower die, as indicated at 11 in Fig. 1, so that the displacement of metal is reduced to the minimum. 65 The empty molds are cooled for reservice by 70 passing them through a cooling tank 12.

The balls 13 are ejected from the die in any appropriate manner, and use is made of their residual heat to toughen or harden them by, for example, treating them in a 75 tank 14. After quenching the residual heat, the balls are transferred to a car 15 through the medium of an endless elevator 16.

Having described the nature and objects of my invention, I claim,—

1. A continuous method of making grinding bodies at one heat, which consists in casting a slug having a substantial part thereof of the ultimate shape of the finished product, forging the slug, while hot from the heat of casting, to the ultimate form desired, and rapidly cooling the forged product.

2. A continuous method of making grinding balls at one heat, which consists in pouring molten metal to form a slug which is in part spherical and in part of displaceable form, the latter containing enough metal to complete the ball, and then forging the slug.

3. A continuous method of making grinding balls, which consists in pouring molten metal to form a slug having a portion thereof of the ultimate shape of the finished product, and having a displaceable portion, forging the slug to ball shape, and utilizing the residual heat of the ball to harden it.

4. A continuous method of making grinding balls at one heat, which consists in pouring molten metal to form a slug which is in part spherical and in part frusto-conical in form, the latter containing enough metal to complete the ball, and then forging the slug.

5. A continuous method of making grind-

2

ing bodies at one heat, which consists in casting a slug having a substantial part thereof of the ultimate shape of the finished product, and having a predetermined displaceable portion of less diameter, forging the slug while hot from the heat of casting to the ultimate form desired, and utilizing the residual heat in appropriate heat treatment of the forged product.

10 6. A slug for use in forming a grinding body, consisting of a casting having a major portion of the ultimate shape of the grind-

ing body and having an offset displaceable portion containing sufficient metal to complete the grinding body without flashing.

7. As an article of manufacture, a commercial grinding body consisting of an integral element whereof the major portion is shaped by casting and whereof the remaining portion is shaped by working; said grinding body being toughened by quenching the residual heat of the casting.

15 In testimony whereof I affix my signature.  
GEORGE R. HANKS.